

## 1

3,074,830

COMBUSTION MIXTURES CONTAINING  
GUANIDINE NITRATECecil A. Rassier, 177 West St., Erith, Kent, England  
No Drawing. Filed Jan. 5, 1960, Ser. No. 481  
5 Claims. (Cl. 149—2)

The present invention relates to composition for generating gas for the purpose, inter alia, of actuating gas pressure operated devices such for instance as the propulsion of rockets and as the gas generative source for reaction motors.

As generating charges are already known which on local heating are capable of maintaining non detonating decomposition these charges comprise mixtures in compacted form containing guanidine nitrate and a poly-nitro- or poly-nitroso-derivative of phenol or of a hydroxy-nitro, carboxy- or methyl substitution derivatives of phenol in which the guanidine nitrate is present in proportions predominating over the total proportions of the other constituents and the phenol derivative is present in sufficient proportion to render the compact mixture capable of sustaining its own non-detonating decomposition once initiated.

Whilst such gas generating charges may be suitable for rocket propulsion and purposes such as blasting operations and dispersion of volatilisable materials or the like they are not wholly satisfactory for purposes where it is highly desirable that the decomposition is uniform throughout the decomposition period with no excessive local over-heating within the charge.

An object of the present invention is to provide a gas generating charge preferably in compacted form which burns regularly to produce throughout its burning life a substantially even gas generation and homogeneous decomposition at a substantially steady temperature.

Broadly the invention comprises a gas generating charge comprising mixtures preferably in granular or compacted form which include guanidine nitrate or similar amidic derivatives of carbonic acid, at least one oxidising salt, and a catalyst which serves to control and to modulise the burning.

Conveniently fillers and/or bonding agents may be incorporated, for example kaolin or china clay or wood flour.

The invention has particular application for use as the fuel in reaction motors, particularly small reaction motors of the type used in toy or scale aircraft or other vehicles, where it is desired to have an even thrust throughout the length of burning without any excessive local over-heating which would damage the relatively light gauge casing of the motor.

As an example of a suitable mix for this purpose the following is given:

80 to 90 parts guanidine nitrate  
35 to 50 parts potassium dichromate  
.5 to 2 parts of sesquioxide of iron  
1 to 3 parts kaolin or china clay  
All parts being by weight

The china clay or kaolin serves not only as a filler but also as a bonding agent enabling the mixture to be compacted by pressure without the inclusion of any separate bonding agent. In addition to bonding agents binding agents may also be employed to give adhesion between the particles in the pellet or charge. By varying the amount of filler the duration of burning can be controlled within certain limits.

Whilst it has been found that for the purpose stated sesquioxide of iron is at this date a preferred catalyst

## 2

which ensures substantial completion of the decomposition of the guanidine nitrate other materials may also be used for example vanadium pentoxide or other vanadate or certain compounds of molybdenum.

5 Furthermore there may be included into the mixtures small amounts of heat resisting materials in addition to clay or kaolin such for example as asbestos fibre which functions solely as a heat resisting material and not as a bonding agent.

10 In addition small quantities of a material such as potassium nitrate or potassium permanganate can be introduced up to .5 part by weight since these compounds serve to produce more complete combustion.

Conveniently the mixture is ground to a suitably small 15 mesh size. The actual grain size used in the mixture depends upon the purpose for which the gas generating charge is required and the rate of burning and consequent rate of gas production and pressure created. It has been found that preferably the oxidising salt and the catalyst 20 should be ground to a finer size than the guanidine nitrate and the grain size chosen is largely determined by the burning rate desired, the smaller the grain size the higher the speed of burning.

With pellets made in accordance with the present invention the burning temperatures can be in the region of 25 1200 to 1300° C. and the fuel burns satisfactorily i.e. at a steady rate up to pressures of 100 lbs. per square inch.

The mixtures of the present invention can be used more 30 particularly in the compacted form as pellets or blocks in a large variety of sizes and can be stored safely without danger of spontaneous combustion or accidental ignition otherwise than, of course, by a proper ignition temperature. Conveniently the pellets may be coated with 35 a thin film of inflammable lacquer for example nitro cellulose which facilitates their handling without crumbling or fracture and at the same time the film is burnt away when the pellet is fired.

Whilst the invention has particular application for use 40 in miniature gas reaction motors because the casing of these motors are usually made of aluminium or aluminium alloy in order to save weight and the mixtures of the invention have the advantage that local overheating is avoided the mixtures may be used for any other purpose where gas production and gas dissemination is required and additional agents may be added to the mixture, for example to increase the burning temperature or to give any other effect required. Thus colouring materials or dyestuffs can be added to the mixture to give off 50 a distinctively coloured combustion gas.

What I claim is:

1. A fuel for generating gas for operating gas pressure-operated devices consisting essentially of a mixture in compacted form of guanidine nitrate 80 to 90 parts by 55 weight, potassium dichromate 35 to 50 parts by weight and sesquioxide of iron 0.5 to 2 parts by weight, the said potassium dichromate and sesquioxide of iron being present in particle size smaller than the particle size of said guanidine nitrate.

60 2. A fuel according to claim 1 in which a bonding agent is present selected from the group consisting of kaolin, china clay and wood flour.

3. A fuel according to claim 1 in the form of a compacted pellet.

65 4. A fuel according to claim 1 in the form of a compacted pellet having a complete protective coating of a combustible lacquer.

5. A fuel according to claim 1 in the form of a compacted pellet having a complete protective coating of a 70 combustible lacquer in the form of a film of nitro-cellulose lacquer.

(References on following page)

References Cited in the file of this patent

## UNITED STATES PATENTS

2,159,234 Taylor ----- May 23, 1939  
2,597,641 Hull et al. ----- May 20, 1952  
2,637,274 Taylor et al. ----- May 5, 1953  
2,740,702 Mace ----- Apr. 3, 1956

2,923,612 Harrison et al. ----- Feb. 2, 1960  
2,925,942 Schmidt et al. ----- Feb. 23, 1960

## OTHER REFERENCES

5 Chemistry and Engineering News, Oct. 7, 1957, pp. 62-63. (Copy in Scientific Library.)